

J. G. HODGSON.  
PROCESS OF MANUFACTURING LACQUERED OR PROTECTIVE COATED CANS.  
APPLICATION FILED APR. 8, 1907.

Patented July 18, 1911.

998,176.



Witnesses:

Wm. Geiger  
H. M. Wenzel

Inventor  
John G. Hodgson.

By Munday, Poore, Adair & Clarke.

Attorneys

# UNITED STATES PATENT OFFICE.

JOHN G. HODGSON, OF MAYWOOD, ILLINOIS, ASSIGNOR TO AMERICAN CAN COMPANY, OF NEW YORK, N. Y., A CORPORATION OF NEW JERSEY.

## PROCESS OF MANUFACTURING LACQUERED OR PROTECTIVE-COATED CANS.

998,176.

Specification of Letters Patent. Patented July 18, 1911.  
Application filed April 8, 1907. Serial No. 366,948.

To all whom it may concern:

Be it known that I, JOHN G. HODGSON, a citizen of the United States, residing in Maywood, in the county of Cook and State of Illinois, have invented a new and useful Improvement in Processes of Manufacturing Lacquered or Protective-Coated Cans, of which the following is a specification.

My invention relates to improvements in the art or process of manufacturing sheet metal preserving cans of tin plate, having soldered end seams uniting the top and bottom heads to the body of the can, and which are provided with lacquer or other protective coating on the inside to keep the food or other products within the can from direct contact with the tin plate and with the solder upon the inside of the can at the soldered end seams or joints thereof. Heretofore sheet metal preserving cans having lacquer or protective coatings on the inside and made with soldered end seams have been made by spraying the lacquer or protective coating over the inside surface of the can after the can is made up, and then subsequently baking or drying the lacquer or protective coating upon the inside of the cans by placing the cans in an oven or heated retort, and subjecting them to a baking and drying heat, usually about 300 degrees Fahrenheit for a period of eight or ten hours or such matter. This old method is slow and expensive in operation, and results in the production of defective and unsatisfactory lacquered or protective coated cans, as it is very difficult by a spraying operation to coat the inside surface of the can evenly and perfectly throughout, and with a coating of uniform thickness, and also because the liquid coating tends to flow or collect at certain portions of the can, and also because it is very difficult to perfectly dry and harden the coating upon the inside of a can where the coating happens to be a little too thick.

The object of my invention is to provide a simple and efficient method or process of rapidly and cheaply manufacturing sheet metal preserving cans having soldered end seams and inside protective coatings by means of which the objections heretofore experienced may be entirely obviated or overcome and the cans be uniformly pro-

duced with perfect or complete interior protective coatings, and by means of which also the tendency of the solder in soldering the end seams of the cans may be prevented from flowing or extending into the can and coating or smearing any portion of the interior surface of the can.

My invention consists in the method or process I have devised, for practically accomplishing this object or result as herein described. That is to say, it consists in first coating in circular spots or areas, the sheets of tin plate from which the can heads are to be cut and formed, with lacquer or other protective coating, the coated spots or areas corresponding in size and shape to the flat or disk portion of the can heads to be cut and formed from the sheet, leaving the portion thereof which forms the flange of the can head uncoated; then baking or drying the sheets, then cutting or forming the can heads from the tin plate sheets having such protective coating in can head spots or areas thereon, then applying the can heads so formed to the can body and then soldering the end seams in the usual manner. By this method or process, the protective coating upon the inside surface of the can head, except the flange thereof which has to be soldered to the can body, serves also to prevent the solder in the soldering operation from flowing into the can and coating or smearing the inside surface of the can adjacent to the soldered end seam. The can bodies or the blanks from which they are formed, whether the can bodies are seamless or made with a side seam, are also provided with an inside coating of lacquer or other suitable material. The can caps for closing the stud holes or filling openings in the tops or upper heads of the cans are also provided with a protective coating excepting at the annular seaming flange thereof, in the same manner and in the same method employed for making the protective coated can head itself.

In the accompanying drawing forming a part of this specification, Figure 1 is a plan view showing a sheet of tin plate having can head spots or areas thereon provided with lacquer or protective coatings according to my invention. Fig. 2 is a sectional view of one of the can heads after the same has been

2  
cut from the sheet of tin plate. Fig. 3 is a sectional view of a protective coated can cap made according to my invention. Fig. 4 is a sectional view showing a can after the can heads have been applied to the body thereof, but before the soldering operation. Fig. 5 is a similar view after the soldering operation or step. Fig. 6 is a sectional view showing the completed can after the cap has been applied and soldered thereto, this view indicating a filled can. Fig. 7 shows a can body blank from which the can body may be formed, if the can body employed is of the kind having a soldered side seam.

15 In the drawing, A represents a sheet of tin plate from which the can heads are to be cut.

$A^1$  represents a series of can head spots or areas and  $A^2$  can cap spots or areas of the sheet having applied thereto a protective coating of lacquer or other suitable material  $a$ , the lacquer or protective coating  $a$  covering the disk portion of the can head, but not extending over the annular portion  $a^1$  thereof which forms the can head flange that encircles the can body and is to be soldered thereto, or over the can cap flange portion  $a^2$  thereof.

B represents the can head, C the can body, the same being either of the seamless kind or of the kind having a lap or lock side seam, as may be preferred. The protective coating  $a$  of the can head does not extend over or cover the flange  $b$  of the can head so that the tinned inner surface of the can head flange which is to be soldered to the end of the can body may come in direct contact with the tinned exterior surface of the can body at the end thereof to facilitate the soldering operation.

40 The can body C is provided with a protective coating  $a$  of lacquer or other suitable material.

The can cap D has a flaring flange or rim  $d$  and the protective coating  $a'$  of the can cap extends only to the inner portion of the flange  $d$ , thus leaving the annular surface of the flange  $d$  uncovered by the coating so that the cap may be readily soldered to the top 45 head of the can by solder  $b^1$ .

50 If the can body C is not made seamless, but made with a soldered side seam, the can body blank from which it is formed is pref-

erably left with a narrow seaming strip  $f$  which has no lacquer or protective coating  $a$ . 55

I claim:

1. The process of manufacturing sheet metal preserving cans having lacquered or protective coatings on the inside thereof, and soldered side, end and cap seams consisting in first coating the sheets of tin plate in the flat in can-body, can head and can cap areas or spots (excepting the portions thereof from which the head and cap flanges and body seam are formed) with a protective coating, then drying and baking the sheets, then cutting and forming the can bodies, can heads and can heads having cap openings therein and can caps therefrom, then forming the body blanks into can bodies and soldering the side seams thereof, then applying the can heads to the can bodies and soldering the end seams thereof and finally applying the caps to the can heads and soldering the cap seams thereof, 75 said protective coating extending to the inner edge of said seams and preventing the solder from extending to the interior surface of the can, substantially as specified.

2. The process of making protective 80 coated can heads with cap openings therein, and with uncoated soldering flanges consisting in applying to a sheet of tin plate in the flat, a protective coating at annular areas thereof from which the can heads are to be 85 cut, and leaving inner and outer flange portion areas uncoated adjacent to each annular coated portion, then drying the coating, then cutting the can heads from the sheet and forming the can heads with cap openings therein and with inner and outer annular flanges, said inner and outer annular flanges being formed from the uncoated annular portions adjacent to each annular 90 coated portion of the sheet, said protective 95 coating extending to the inner edge of the lapping portions of said inner and outer annular flanges and serving to prevent the solder from extending to the interior surface of the can when the cap is soldered to 100 the can head, substantially as specified.

JOHN G. HODGSON.

Witnesses:

EDMUND ADCOCK,  
H. M. MUNDAY.